

Aug. 28, 1962

**E. GORIN ET AL**  
PREPARING METALLURGICAL FUEL FROM NON-CAKING  
COAL UTILIZING AIR-BLOWN PITCH BINDER  
Filed July 22, 1960

3,051,628

Filed July 22, 1960



INVENTORS.  
EVERETT GORIN  
ROBERT J. FRIEDRICH

BY

BY  
*D. Leigh Fowler, Jr.*  
ATTORNEY

## 1

3,051,628

## PREPARING METALLURGICAL FUEL FROM NON-CAKING COAL UTILIZING AIR-BLOWN PITCH BINDER

Everett Gorin, Pittsburgh, and Robert J. Friedrich, Finleyville, Pa., assignors to Consolidation Coal Company, Pittsburgh, Pa., a corporation of Pennsylvania

Filed July 22, 1960, Ser. No. 44,602  
4 Claims. (Cl. 202—26)

The present invention relates to the preparation of metallurgical fuel from non-caking and weakly caking bituminous and sub-bituminous coal.

The present application is a continuation-in-part of our copending application Serial No. 746,990, filed July 7, 1958, and assigned to the assignee of the present invention.

There are substantial reserves of non-caking coals throughout the world which, because of their non-caking property, cannot be converted into metallurgical fuels by conventional coking processes. Attempts have been made to utilize non-caking coals in the production of metallurgical coke by a process sequence involving: first, low temperature carbonization of the coal to yield a solid distillation residue known as char; second, briquetting the resulting char with suitable binders; and third, coking and calcining the prepared briquets. Coke produced in this manner has been too weak for metallurgical use. The weakness of such coke can be attributed to the differential shrinkage of the char particles away from the briquet binder which occurs during the calcining of the briquets. Addition of substantial quantities of strongly caking coal into the briquet formulation yields coke of satisfactory strength. However, the addition of strongly caking coal is not a generally satisfactory expedient because of its relatively high cost and non-availability in geographical areas where non-caking coal is found.

A typical non-caking coal available in Wyoming has the following analysis:

TABLE I

*Properties of Typical Non-Caking Coal*

| Proximate analysis:                      | Weight percent |
|------------------------------------------|----------------|
| Moisture                                 | 19.20          |
| Volatile matter                          | 38.44          |
| Fixed carbon                             | 39.68          |
| Ash                                      | 2.68           |
| Ultimate analysis (moisture-free basis): | Weight percent |
| H                                        | 5.02           |
| C                                        | 74.41          |
| N                                        | 1.28           |
| O                                        | 15.04          |
| S                                        | 0.93           |

The high percentage of oxygen in the coal is characteristic of non-caking coals. Non-caking coal, when heated to elevated temperatures, merely crumbles and evolves gases and tar vapors. It does not soften to form agglomerate particles which would form a strong cellular coke, but instead leaves a soft powdery mass as a residue. Numerous well-known tests have been developed to distinguish caking coals from non-caking coals. Lowry, "The Chemistry of Coal Utilization," vol. I (1945), pages 73, 77-79.

Non-caking coal can be comminuted to a fluidizable size and carbonized at low temperature (850 to 1100° F.) to produce gas, tar and a char residue. Because the starting coal is non-caking, no preliminary decaking treatment is required and hence substantial tar yield can be achieved.

By preliminarily shrinking the char from a non-caking

## 2

coal prior to briquet formation, the adverse effects of differential shrinkage can be avoided and coke of satisfactory strength can be prepared. The char can be shrunk by heating it to an elevated temperature at which particle contraction occurs. This elevated temperature of shrinking will be above the temperature at which the char was generated from the starting coal, and, in general, will be in the range of 1350 to 1800° F. The shrinking treatment is accompanied by devolatilization of the char which yields substantial quantities of combustible gases rich in hydrogen and methane.

It is possible to prepare coked briquets of satisfactory metallurgical strength by directly carbonizing, devolatilizing and shrinking the non-caking coal in a single high temperature carbonization treatment. However, the yield of tar from high temperature carbonization is inadequate to provide autogenously the pitch binder requirements of the subsequent briquet formulation. Low temperature carbonization at temperatures from about 800 to 1100° F. maximizes the yield of tar and assures the provision of the required amount of pitch binder. However, the pitch obtained directly from low temperature carbonization of a non-caking or weakly caking coal, unfortunately, does not possess satisfactory binder properties for briquet formulations. While resort may be had to other materials to serve as binders. It would be highly desirable from an economic standpoint to obtain a suitable binder from the coal utilized as feed to the briquetting operation.

Accordingly, the primary object of this invention is to provide a process for making strong briquets from a non-caking or weakly caking coal, wherein essentially all the requisite ingredients of the briquets are derived from the coal itself.

Another object of this invention is to provide a process for making a suitable binder for briquet formulations from a non-caking or weakly caking coal.

Other objects and advantages of our invention will become apparent upon reference to the following description and to the accompanying drawing in which there is shown a schematic flow diagram illustrating apparatus adapted to the practice of the invention.

In accordance with the present invention, we are able to make strong briquets solely from ingredients derived from a non-caking coal. Our process briefly comprises carbonizing the coal at low temperatures to yield char and tar. The char is further heated to an elevated temperature to effect shrinkage. The tar is fractionated to recover high boiling pitch, middle distillate oil, and a low boiling fraction. The pitch is blown with air at elevated temperature to increase its fixed carbon content to 25 to 50 percent. A portion of the middle distillate oil may be blended, if necessary, with the air blown pitch to reduce the melting point of the pitch. The resulting blend is mixed with the preshrunk char and formed into raw briquets which are thereafter calcined to yield a strong briquet as product.

Referring now to the drawing for a description of the preferred embodiment of our invention, the principal apparatus includes a coal crusher 10, a fluidized coal dryer 11, a fluidized low temperature carbonization vessel 12, a surge vessel for product char 13, a briquet calcining vessel 14, a hot char quenching vessel 15, a kneading apparatus 16 for briquet formulation, a briquet making apparatus 17, a tar condenser 18, a tar decanter vessel 19, a tar distillation vessel 20, a pitch air blowing vessel 21 and a briquet binder mixing vessel 22.

The starting coal is introduced into the coal crusher 10 where it is comminuted to a fluidizable size, for example, capable of passing through a 14-mesh Tyler Standard

screen. A typical particle size distribution (wet screen analysis) for a comminuted non-caking coal is:

TABLE II  
Particle Size Distribution

| Tyler screen sizes:     | Weight percent |
|-------------------------|----------------|
| On 14 mesh              | 0.0            |
| Through 14 on 28 mesh   | 17.1           |
| Through 28 on 48 mesh   | 31.1           |
| Through 48 on 100 mesh  | 23.9           |
| Through 100 on 150 mesh | 8.1            |
| Through 150 on 200 mesh | 5.2            |
| Through 200 on 325 mesh | 6.0            |
| Through 325 mesh        | 8.6            |

Suitably comminuted non-caking coal is recovered from the coal crusher 10 and transferred through a conduit 23 into the fluidized coal dryer 11. Hot gases for fluidizing and drying the coal are generated in a combustion vessel 24 and by combustion of fuel gas with air introduced through conduits 25 and 26 respectively. The hot combustion gases are transferred through a conduit 27 for drying and preheating the comminuted coal in the dryer 11. Since the coal is non-caking, the dryer 11 may also serve as a preheater. Accordingly, the coal is not only dehydrated but also preheated in the dryer 11 to a temperature of about 300-600° F. The spent fluidizing gases are removed from the dryer 11 through a conduit 28. Preferably any entrained solids in the spent fluidizing gases are recovered by passing the gases from the conduit 28 through suitable recovery equipment.

Preheated dehydrated coal is recovered from the dryer 11 through a conduit 29 and is introduced into the fluidized low temperature carbonization vessel 12. The coal is maintained in a fluidized state in the fluidized low temperature carbonization vessel 12 at a temperature of about 800 to 1100° F. (preferably about 850 to 950° F.). Air, employed as the fluidizing gas, is introduced through a conduit 30. The coal is maintained in the low carbonization vessel 12 for about 10 to 60 minutes until substantially complete tar evolution has occurred. Gases, tar vapors and oxygen-depleted air are recovered through a conduit 31 and are transferred to the tar condenser vessel 18 for further treatment to be hereinafter described.

The heat required for carbonization is supplied by partial combustion of the coal with the oxygen content of the fluidizing air. Because of the non-caking property of the starting coal, there is no tendency for particle size agglomeration. Accordingly, the product char, recovered through a conduit 32, has a free-flowing particulate character.

The product char is transferred without deliberate cooling through the conduit 32 into the product char surge vessel 13. The char is maintained within the surge vessel 13 substantially at the carbonization temperature. One portion of the product char is withdrawn through a conduit 33 and introduced into a char burner 34 for turbulent contact therein with air from a conduit 35. The partially burned char and air are transferred at an elevated temperature as a dilute phase suspension from the burner 34 into a transfer conduit 36. The remainder of the char from the surge vessel 13 is withdrawn through a conduit 33a and introduced into the transfer conduit 36 to supplement the dilute phase suspension of heated char and air. The final temperature of the dilute phase stream must be sufficient to effect the desired char shrinking, i.e., from about 1350 to 1800° F. Hence the air and char stream leaving the char burner 34 should be at a temperature of about 1600 to 2250° F. The preshrinking treatment of the char permits production of briquets therefrom which will possess satisfactory high temperature strength following suitable calcining treatment. Heating of the char to temperatures above

the carbonization temperature at which it was generated results in further devolatilization of the char yielding significant quantities of combustible devolatilization gases rich in hydrogen and methane.

The calcining treatment for briquets occurs within the calciner vessel 14. Cold, freshly produced briquets are introduced into the top of the calciner vessel 14 through a conduit 37. The briquets pass downwardly through the calciner vessel 14 and are contacted with the dilute phase suspension of hot preshrunk char in hot gases. The preshrunk char and gases are cooled and the briquets are heated by heat interchange within the calciner vessel 14. The briquets, following calcining, are withdrawn from the bottom of the calciner vessel 14 through a conduit 38 at a temperature between 1400 and 1700° F., preferably about 1600° F. The final briquet temperature, of course, is lower than the temperature of the dilute phase suspension of shrunk char and gases which enters the calciner vessel 14 through the transfer conduit 36.

The fresh briquets which enter the calciner vessel 14 are at first heated very rapidly, i.e., shock-heated, by virtue of their sudden exposure to the elevated temperatures therein. Thereafter the briquets are more slowly heated to calcining temperatures. The residence time of the briquets in the calciner vessel preferably is from about one-half to two hours. This rapid initial heating serves to coke the briquet binder quickly and to set the binder as a matrix for confining the char particles. Appreciable quantities of tar vapors are evolved during this coking. The tar vapors are carried along with the heated gases and entrained shrunk char. The dilute phase suspension of shrunk char is recovered from the top of the calciner vessel 14 through a conduit 39. The shrunk char is recovered in a cyclone separator 40 and transferred through a conduit 41 into a quench vessel 15. The hot gases and tar vapors, substantially free of entrained shrunk char particles, are recovered from the cyclone separator 40 through a conduit 42 and are introduced into the tar condenser vessel 18 along with the primary carbonization tar vapors for further treatment as will be hereinafter described.

The shrunk char particles are cooled in the char quench vessel 15 to a temperature of about 500° F. Suitably, the carbonization liquor can be sprayed into the quench vessel 15 to quench the hot char particles while extracting the volatilization heat of the liquor. The quenched char is recovered at about 300 to 400° F. from the char quench vessel 15 through a conduit 43 and introduced into the briquet kneading apparatus 16. Suitable quantities of pitch binder are introduced into the briquet kneading apparatus 16 through a conduit 44. The mixture of hot char and pitch binder is kneaded in accordance with conventional briquet making procedures, i.e., at a temperature about 40° F. above the melting temperature of the binder pitch.

The kneaded mixture of char and pitch binder is recovered from the kneading apparatus 16 and introduced into briquet making apparatus 17 wherein the mixture is pressed at suitable mechanical pressures into uniform shapes preferably from 1/2 to 3 inches in maximum transversal dimension. Formed briquets are recovered from the briquetting apparatus and transferred through a conduit 37 to the calciner vessel 14 as already described. It is customary in briquetting practice to provide slight cooling of the fresh briquets below the melting point of the binder pitch before they are subjected to vigorous mechanical movement.

The present process autogenously provides the required pitch binder from the tar which is inherently produced. This process will be briefly described. Referring to the tar condenser vessel 18, tar vapors and non-condensable gases introduced through conduit 31 are quenched by a recirculating liquid spray introduced through a conduit 45. The liquid spray preferably is the

carbonization liquor. Non-condensable gases are recovered overhead through a conduit 46. The non-condensable gases may be burned to provide the hot gases required for the coal dryer 11. The condensable tar products are recovered along with the condenser spray liquid through a bottom conduit 47. The condensed liquids are separated in a decanter vessel 19. Supernatant aqueous liquids are recovered and recirculated through the conduit 45 to the condenser vessel 18. Condensed liquid tar is recovered through a conduit 48 and introduced into a distillation vessel 20 for separation. The valuable low boiling tar components, e.g., those boiling below about 230° C., are recovered as a distillate product through a conduit 49. A middle boiling tar distillate, for example, boiling from about 230 to 350 or 375° C., is recovered through a conduit 50. The high boiling pitch components, for example, those boiling above about 350 to 415° C., are recovered as a bottom product through a conduit 51.

Freshly prepared pitch from non-caking coal has been found to be unsatisfactory as a briquet binder. However, it can be employed as a pitch binder if subjected to a preliminary air blowing treatment at elevated temperatures, for example, 500 to 900° F. The air blowing should be carried out at a sufficient pressure to avoid volatilization of the pitch components. Accordingly, the pitch is transferred from the conduit 51 into the air blowing vessel 21 maintained at an elevated temperature. Air is introduced into the air blowing vessel 21. The pitch is contacted with air for about 20 minutes. An air blown pitch product, suitable as a briquet binder, is recovered through a conduit 52. The solids-free pitch should have a fixed carbon content (Conradson Carbon) between 25 and 50 percent.

The air blown pitch binder recovered through the conduit 52 may have an excessive melting point. It is desirable that the pitch should become molten at briquet kneading temperatures in order to wet the char particles completely during the kneading treatment which is customarily carried out with steam heat. Hence the pitch may be blended with middle boiling tar distillate to provide a suitable melting point binder for use in briquet making. A melting point of about 90 to 120° C. is preferred. Accordingly, a portion of the middle boiling tar distillate is withdrawn from the conduit 50 and transferred through a conduit 53 to the binder mixing vessel 22 for blending with air blown pitch to produce a pitch binder of satisfactory melting properties for use in briquet formulations. The binder pitch tends to be unstable when stored in liquid form. Hence it is cooled below its melting temperature and stored as a solidified mass. Prior to use, the solid pitch is comminuted and blended into the briquet formulation as solid particles.

#### EXAMPLE

The following example is presented to illustrate a material balance and operating conditions for a briquet making plant as illustrated in the drawing. The following data are derived from a briquet plant processing 50 tons per hour of non-caking coal having the properties listed in Table I. The coal is preliminarily crushed to the size distribution listed in Table II.

The coal is introduced into a fluidized dryer 11 maintained at a temperature of 400° F. 33,000 cubic feet per minute of gases at 205° F. are recovered from the dryer through conduit 28 containing 510 pounds of entrained solids. 80,420 pounds per hour of dried preheated coal at 400° F. is introduced into a fluidized carbonization vessel 12 and maintained therein for 30 minutes. 4,750 cubic feet per minute of air is introduced into the carbonization vessel through a conduit 30 as fluidizing and partial combustion gas. A temperature of 925° F. is maintained within the carbonization vessel. The linear velocity of the fluidizing gases is about 1.65 feet per second.

The carbonization gases, recovered through conduit 31, include:

|             | Pounds per hour |
|-------------|-----------------|
| Dry tar     | 12,110          |
| 5 Solids    | 3,600           |
| Gas         | 26,000          |
| Water vapor | 8,380           |

50,500 pounds per hour of char at 925° F. is introduced into a char surge vessel 13. The char has the following analysis:

TABLE III  
*Char Properties*

|    |                                                 |                |
|----|-------------------------------------------------|----------------|
| 15 | (A) Proximate analysis:                         | Weight percent |
|    | Volatile matter                                 | 22.22          |
|    | Fixed carbon                                    | 72.74          |
|    | Ash                                             | 5.04           |
| 20 | (B) Ultimate analysis:                          |                |
|    | H                                               | 3.16           |
|    | C                                               | 79.94          |
|    | N                                               | 1.36           |
|    | O                                               | 9.69           |
|    | S                                               | 0.81           |
| 25 | (C) Particle size distribution<br>(wet screen): |                |
|    | On 14 mesh                                      | 0.0            |
|    | Through 14 on 28 mesh                           | 10.2           |
|    | Through 28 on 48 mesh                           | 27.4           |
| 30 | Through 48 on 100 mesh                          | 29.8           |
|    | Through 100 on 150 mesh                         | 13.1           |
|    | Through 150 on 200 mesh                         | 6.1            |
|    | Through 200 on 325 mesh                         | 8.5            |
| 35 | Through 325 mesh                                | 4.9            |

It is apparent that substantially no agglomeration occurs during carbonization when the particle size analysis of the product char (Table III) is compared with that of the starting coal (Table II).

40 28,600 pounds per hour of char from conduit 33 are partially burned with 5,680 standard cubic feet per minute of air from conduit 35 to produce a dilute phase suspension of hot char in combustion gases at a temperature of about 2200° F. This dilute phase suspension is blended with 21,900 pounds per hour of char from conduit 33a to produce a dilute phase stream of char suspended in gases in the conduit 36 at a temperature of about 1800° F. At this temperature, the char is further devolatilized and experiences a shrinking to effect increased strength. 45 The entire steam of char and hot gases is blown upwardly through a calciner vessel 14. 61,500 pounds per hour of raw briquets are introduced into the top of the calciner vessel. By interchange of heat, the briquets leave the bottom of the calciner vessel at a temperature of about 50 1650° F. and are cooled to produce 52,050 pounds per hour of dry coke. The shrunk char and hot gases are cooled via heat interchange within the calciner vessel to a temperature of 740° F. and withdrawn through a conduit 39. The bulk of the entrained shrunk char is recovered from a cyclone separator 40 and introduced into 55 a quench drum 15 where it is cooled to about 490° F. for subsequent use in briquet formulation. The effluent stream, recovered through a conduit 42, from the cyclone separator 40 comprises:

|    | Pounds per hour |        |
|----|-----------------|--------|
| 65 | Dry tar         | 8,180  |
|    | Solids          | 4,260  |
|    | Gas             | 30,200 |
|    | Moisture        | 5,290  |

70 This effluent stream is blended with the carbonization effluent gases and introduced into a condenser 18.

The blended vapor stream recovered from the calciner and carbonization vessel is quenched by water spray to a temperature of about 170° F. The non-condensable gases are recovered at a temperature of about 90° F. and com-

prise 59,000 pounds per hour of gas having a net heating value of about 208 B.t.u. per cubic foot. The condensed tar product includes 20,300 pounds per hour of dry tar, 7,860 pounds per hour of entrained solids and 1,185 pounds per hour of moisture. The tar is dehydrated to remove the moisture and introduced into a distillation tower 20 at a temperature of about 720° F. The pitch product boiling above 415° C. contains 9,080 pounds per hour of pitch and 7,860 pounds per hour of entrained solids. This material is introduced into an air blowing vessel 21 maintained at 710° F. About 90 standard cubic feet per minute of air is blown into the air blowing vessel and the effluent vapors are recombined with the lower boiling distillate fractions of the tar. The product air blown pitch, recovered through conduit 52, comprises 8,010 pounds per hour of pitch and 7,860 pounds per hour of entrained solids. This material is blended with 4,210 pounds per hour of middle tar distillate from conduit 53 having a boiling range between 300 and 415° C.

Thus a total of 20,100 pounds per hour of briquet binder pitch is produced and is cooled to solidification. The solid pitch is comminuted to simplify its subsequent blending with product char in the briquet formulation. The small quantity of coal which was entrained in the dryer effluent conduit 28 (510 pounds per hour) preferably is also combined into the briquet formulation. In addition, the fine particles of product briquets resulting from abrasion are recovered by screening and are incorporated in the briquet formulation. Typically these briquet recycle fines will amount to 5,720 pounds per hour.

The shrunk char, recycle coke fines, coal fines from the dryer and pulverized binder pitch are introduced into a briquet kneader at about 260° F., i.e., slightly above the melting point of the pitch binder. The briquets are pressed in a briquet making apparatus 17 and cooled below the pitch melting point for mechanical strength. A total of 61,500 pounds per hour of raw briquets results. These are the briquets which are introduced into the calciner vessel 14 for coking.

#### FURTHER EXAMPLES

The following tests are reported herein to illustrate the effects, respectively, of preliminary char shrinking and of air blown pitch on product metallurgical coke obtained from non-caking coal.

*Test 1.*—A briquet formulation was prepared according to the present invention. A binder pitch was produced from the low temperature carbonization pitch boiling above 375° C. The pitch was air blown to a fixed carbon value of 38 percent by weight. The pitch was blended with middle boiling tar distillate (300 to 375° C.). Char from fluidized low temperature carbonization of non-caking coal was heated to 1800° F. to effect shrinking. The briquet formulation was as follows:

|                       | Parts |
|-----------------------|-------|
| Preshrunk char        | 80.7  |
| Air blown pitch       | 11.0  |
| Middle tar distillate | 8.3   |

One-inch briquets prepared from this formulation, when coked to 1800° F., showed a Tumbler Index of 95.8 (when quenched in nitrogen gas) and 94.5 (when quenched in water). Thus briquets of acceptable strength can be prepared according to this invention. The Tumbler Index is similar to that described in ASTM Test Designation D 294-50, modified to provide for the one-inch diameter briquets.

*Test 2.*—The same pitch binder and middle boiling tar distillate were combined with char obtained from fluidized low temperature carbonization of the same non-caking coal used in Test 1. The char was not preshrunk, but instead was formulated into briquets without intervening thermal treatment. The briquet formulation was as follows:

|                       | Parts |
|-----------------------|-------|
| Char                  | 86.0  |
| Air blown pitch       | 8.4   |
| Middle tar distillate | 5.6   |

5 The Tumbler Index of the resulting coked briquets was 55.1. Thus the improved coke strength achieved by preliminary char shrinking is clear when the results of Tests 1 and 2 are compared.

*Test 3.*—Briquets were prepared from the same starting ingredients of Test 2 with the addition of a minor portion of caking coal. The caking coal was a Pittsburgh Seam high volatile, strongly caking coal obtained in northern West Virginia. The formulation was as follows:

|                       | Parts |
|-----------------------|-------|
| Char                  | 73.0  |
| Air blown pitch       | 7.1   |
| Middle tar distillate | 5.7   |
| Caking coal           | 14.2  |

20 The Tumbler Index of the resulting coked briquets was 80.0. Hence it is seen that improved briquets can be prepared from the char product of non-caking coal when a minor portion of strongly caking coal is incorporated into the formulation. However, the briquet strength achieved by addition of caking coal to the briquet is not as high as that resulting from the use of shrunk char.

*Test 4.*—Briquets were prepared from a formulation comprising char from fluidized low temperature carbonization of a non-caking coal and a binder pitch produced from the low temperature carbonization pitch boiling above 375° C. The char had been heated to 1800° F. to effect shrinking, but the pitch was not air blown, in contrast to the pitch employed in the first three tests. The formulation was as follows:

|                       | Parts |
|-----------------------|-------|
| Preshrunk char        | 85.0  |
| Pitch (not air blown) | 15.0  |

35 The Tumbler Index of the resulting coked briquets was 85.9. Thus, while the use of preshrunk char effected a substantial improvement, the use of non-air blown pitch prevented attaining the high Tumbler Index obtained in Test 1.

40 While fluidized low temperature carbonization has been described in the foregoing specification as a preferred processing technique, nevertheless, other forms of low temperature carbonization may be employed, preceded or followed by crushing of the solids to a particle size suitable for effective shrinking treatment and heat interchange with pressed briquets.

45 According to the provisions of the patent statutes, we have explained the principle, preferred construction and mode of operation of our invention and have illustrated and described what we now consider to represent its best embodiment. However, we desire to have it understood that, within the scope of the appended claims, the invention may be practiced otherwise than as specifically illustrated and described.

50 We claim:

1. The method of preparing coked briquets from a non-caking coal which comprises carbonizing said non-caking coal to produce gas, tar and char, heating said char in particulate form to an elevated temperature above the carbonization temperature at which said char was generated to effect shrinking of the char, recovering a high boiling pitch from said tar, subjecting said pitch to air blowing at an elevated temperature to thereby increase its fixed carbon content, forming raw briquets from said preshrunk char and said air blown pitch at low temperature, and thereafter coking said raw briquets.
2. The method of preparing coked briquets from a non-caking coal which comprises carbonizing said non-caking coal in a fluidized state at a temperature between about 800 and 1100° F. to produce gas, tar and char, heating said char in particulate form to a temperature between about 1350 and 1800° F. to effect shrinking of

the char, fractionally distilling said tar to recover a pitch boiling above about said 350 to 415° C. and a distillate fraction boiling from about 230 to 375° C., subjecting said pitch to air blowing at a temperature between 500 and 900° F. to increase its fixed carbon content to between 25 and 50 percent, blending said pitch with at least a portion of said distillate fraction to produce a material having a melting point between 90 and 120° C., forming raw briquets from said preshrunk char and said blended material, at a temperature above the melting point of said blended material, and thereafter coking said raw briquets.

3. In the process of preparing coked briquets from char and pitch obtained by the carbonization of a non-caking coal at a low temperature, the improvement which comprises heating said char in particulate form to an elevated temperature above the carbonization temperature at which said char was generated to effect shrinking of the char, subjecting said pitch to air blowing at an elevated temperature to thereby increase its fixed carbon content to between 25 and 50 percent, thereafter incorporating said preshrunk char and said air blown pitch in a briquet formulation, forming

15

20

briquets from said formulation, and thereafter coking said briquets.

4. In the process of preparing coked briquets from char and pitch obtained by the carbonization of non-caking coal at a low temperature, the improvement which comprises heating said char in particulate form to an elevated temperature above the carbonization temperature at which said char was generated to effect shrinking of the char, increasing the fixed carbon content of said pitch to between 25 and 50 percent, thereafter incorporating said preshrunk char and said pitch in a briquet formulation, forming briquets from said formulation, and thereafter coking said briquets.

References Cited in the file of this patent

UNITED STATES PATENTS

|           |               |               |
|-----------|---------------|---------------|
| 2,095,190 | Heuscher      | Oct. 5, 1937  |
| 2,203,645 | Reynard       | June 4, 1940  |
| 2,594,226 | Shea          | Apr. 22, 1952 |
| 2,683,107 | Juel          | July 6, 1954  |
| 2,864,760 | Croy          | Dec. 16, 1958 |
| 2,985,577 | Geller et al. | May 23, 1961  |